

June 24, 1924.

1,499,308

C. E. RAHR

PREPARED ROOFING AND PROCESS OF MAKING SAME

Filed Oct. 5, 1921

Fig. 1.



Fig. 2.



Fig. 3.



Witness,  
S. J. Mann

Inventor,  
Chester E. Rahr.  
By Frank L. Belknap. *7/11/21*

## UNITED STATES PATENT OFFICE.

CHESTER E. RAHR, OF BOSTON, MASSACHUSETTS, ASSIGNOR TO THE FLINTKOTE COMPANY, OF BOSTON, MASSACHUSETTS, A CORPORATION OF MASSACHUSETTS.

## PREPARED ROOFING AND PROCESS OF MAKING SAME.

Application filed October 5, 1921. Serial No. 505,502.

To all whom it may concern:

Be it known that I, CHESTER E. RAHR, a citizen of the United States, residing in the city of Boston, county of Suffolk, and 5 State of Massachusetts, have invented certain new and useful Improvements in Prepared Roofing and Processes of Making Same, of which the following is a specification.

- 10 This invention is more particularly directed to that type of waterproof covering in which symmetrical designs are formed by means of comminuted material. In the present invention the designs are formed by 15 having spaced selected areas of one face of the product covered by comminuted granular or gritty material, such as gravel, green stone, crushed rock, crushed brick or the like, while the main areas are covered by 20 granular comminuted material of a contrasting color to the first comminuted material, the second comminuted material being of an asphaltic or bituminous character.

Among the salient objects of the invention 25 are to provide a waterproofing sheet, the body portion of which consists essentially of asphalt or bituminous saturated felt, one face of which is covered with an adhesive coating and upon which coating is applied 30 two different comminuted materials in the form of symmetrical designs; to produce a product in which the ornamental designs are formed by the combined use of comminuted bituminous asphaltic or pitchy hard bodies 35 of a non-bituminous, granular material; to provide a product in which the bituminous, pitchy or asphaltic bodies may be formed of such substances as gilsonite, elaterite, wurtzilite, Cuban asphalt and in some cases even 40 Cuban, Trinidad or Bermudez asphalt or coal tar or other hard pitches.

In the drawings—

Fig. 1 is a face view of the sheet.

Fig. 2 is an edge view, and

45 Fig. 3 is a fragmentary view of the sheet before surfacing.

Referring in detail to the drawing, the roofing felt 1, such as is common to the prepared roofing art or any fabricated substance used in this connection such as paper stock emulsified with waterproofing bituminous substance coated with an adhesive coating 2 such as asphalt, forms of pitch

or tar or numerous other substances having a bituminous base, is imposed in the form 55 of a coating upon the saturated sheet and is maintained in an adhesive form while a comminuted substance 3 such as asphalt, gilsonite, elaterite, wurtzilite, or comminuted oil shale, dry comminuted refined 60 Trinidad or Bermudez is placed upon the sheet in the form of a design. This design may be made to simulate common shingles or hexagonal forms of prepared shingles or innumerable figures placed upon the coated sheet to produce an ornamental effect. This comminuted substance placed in the 65 form of a design adheres to the coated sheet and produces non-adhesive surface on those portions of the sheet which are covered. After the imposition of this design, there is placed upon the sheet a granular 70 surfacing material 4 such as gravel, crushed stone and slate of distinguishing colors, such as red, green or yellow, which will 75 adhere to the sheet upon the portions which are not covered by the non-adhesive design making substance.

The two materials so placed upon the adhesive sheet produce an attractive ornamented roofing sheet which, when pressure rolled, forms an attractive surfacing which is inexpensive to manufacture and at the same time, has the advantages of the more expensive roof coverings now upon the 80 market. The design shown in the drawings is but one example of innumerable effects that may be produced with the placing of the substances upon the adhesive coated sheet. Similar roofing sheets have been produced where graphite has been used to form 85 the design and a granular substance applied to fill the spaces between the designs. Also roofing material has been produced in which the portion of the sheet has been 90 kept totally devoid of material and the design produced by surfacing only that portion of the sheet which lies between the design markings.

The present product is a departure from 100 this in that a comminuted bituminous or asphaltic substance of substantially higher melting point is imposed upon the sheet in the form of a design and the granular surfacing placed between these design 105 markings as it will not adhere to the non-

adhesive design markings which are placed upon the sheet in the form of the higher melting point substance.

I claim as my invention:

- 5 1. Prepared roofing comprising a sheet saturated with a waterproof composition and coated with an adhesive substance, a comminuted non-adhesive bituminous substance imposed upon the adhesive coating 10 in the form of a design and a colored granular surfacing, covering the adhesive coating not occupied by the non-adhesive design forming substance.
- 15 2. Prepared roofing comprising a sheet of felted fibrous material saturated with a waterproof substance and coated with an adhesive bituminous composition, a comminuted non-adhesive high melting point bituminous substance, placed upon the adhesive coating in the form of a design and a colored granular substance surfacing the adhesive coating on that portion of the sheet not occupied by the non-adhesive substance.
- 20 25 3. A process for producing prepared roofing, consisting in coating a sheet of prepared

roofing with an adhesive substance, imposing a design of non-adhesive comminuted asphaltic substance upon the adhesive coating and surfacing the remaining adhesive 30 coating with a colored granular surfacing.

4. A process of producing prepared roofing, consisting in coating the prepared roofing sheet with an adhesive bituminous composition, producing a design thereon by the 35 imposition of a comminuted high melting point asphaltic composition and surfacing the remaining portion of the sheet with a colored granular mineral surfacing.

5. A process of producing prepared roofing consisting in coating a sheet with a waterproofing adhesive substance, applying a design of non-adhesive high melting point asphaltic material upon the adhesive coating to produce non-adhesive areas of a pre-determined configuration, applying a granular surfacing to the sheet which adheres to the adhesive portion, impressing the granular surfacing into the coating substance whereby a design is produced by the non- 45 50 adhesive areas.

CHESTER E. RAHR.